

## UNITED STATES PATENT OFFICE

2,663,636

ELECTROPHOTOGRAPHIC PLATE AND  
METHOD OF PRODUCING SAME

Arthur E. Middleton, Columbus, Ohio, assignor,  
by mesne assignments, to The Haloid Company,  
Rochester, N. Y., a corporation of New York

No Drawing. Application May 25, 1949,  
Serial No. 95,374

13 Claims. (Cl. 95—1.9)

1

This invention relates to electrophotographic plates and to a method of producing such plates. More particularly, the invention relates to a composition of matter including a photoconducting insulating material and to an electrophotographic plate containing a coating of such composition. Specifically, the invention relates to a method of producing a composition of matter containing a photoconducting insulating material and to a method of making an electrophotographic plate coated with such composition.

In the electrophotographic process, a base plate of low electrical resistance having a photoconducting insulating coating thereon is electrostatically charged in the dark. The charged coating is then exposed to light through a negative photographic film, positive film or mask, or otherwise to a light image, to receive a latent electrostatic image. If the plate has been properly prepared, the charges leak off rapidly to the base plate in proportion to the intensity of light to which any given area is exposed, and after such exposure, powder is dusted on the coating in the dark and adheres to the areas where the electrostatic charges remain, forming a powder image corresponding to the electrostatic image. The powder image can then be transferred to a sheet of transfer material resulting in a positive or negative print as the case may be, having excellent detail and quality.

One object of the invention is to improve the photoconductive characteristics of the plate and insure proper functioning of the plate when exposed, this being accomplished by producing a composition of matter containing a photoconducting insulating material which can be applied as a coating on a base plate in a practical and economical manner, and which adheres firmly thereto and acts successfully as a photoconducting insulating layer.

Another purpose of the invention is to provide a method for coating a base plate at room temperatures with a composition containing a photoconducting insulating material, and which will adhere permanently and securely to the base plate and act efficiently as a photoconducting insulating layer.

A further object of the invention is to provide a composition of matter containing a photoconducting insulating material and which will adhere readily and permanently to a base plate and act as a photoconducting insulating layer.

An additional purpose of the invention is to provide an improved and more efficient electrophotographic plate having on its surface an ad-

2

herent coating comprising a composition containing a photoconducting insulating material, and capable of acting as a photoconducting insulating layer.

5 It has now been found that an efficient electrophotographic plate can be obtained by spraying a base plate at room temperature with a photoconducting insulating composition prepared by intimately mixing and grinding together a photoconducting insulating material, a high electrical resistance binder, and a solvent. On evaporation of the solvent, the composition forms a successful adherent layer on the plate that will hold electrostatic charges in the dark and rapidly lose them on exposure to light.

In general, the invention comprises intimately mixing and grinding together in a ball mill or other suitable fashion a photoconducting insulating material such as pure amorphous selenium with a solvent and a binder material having an electrical volume resistivity of about  $10^{10}$  to about  $10^{19}$  ohms-cm., for a period of time sufficient to insure intimate mixture and reduction of the size of the particles. At the end of the milling period 15 additional solvent may be added and stirred into the mixture sufficiently to render it sprayable. The resulting composition can readily be sprayed at room temperatures onto a clean, unheated base plate. After the solvent has evaporated from the composition, the coating can be electrostatically charged and used in the electrophotographic process.

The selenium must be of the amorphous type and free of impurities such as copper, iron, lead and bismuth which appear to affect adversely its ability to hold electrostatic charges by decreasing its electrical resistance so that the charges leak off rapidly in the dark and powder images cannot be obtained. It is preferred to use amorphous "A. R. Q." selenium (ammonia reduced in quartz from  $\text{SeO}_2$ ) in pellet form, from about  $\frac{1}{16}$ " to  $\frac{1}{8}$ " size, as manufactured by the Canadian Copper Refiners Company Limited, Montreal East, Ontario, Canada, and containing less than about 20 parts per million of impurities.

40 Other grades and types of selenium as furnished commercially can be used if purified and converted into the amorphous state. To obtain essentially purified amorphous selenium from the impure forms, it is the usual practice to first free it of the copper, iron, lead or bismuth by distillation and then to melt down the required amount of selenium in a container exposed to the atmosphere by heating to a temperature of from 250° C. to 300° C., and preferably about 250° C. The

molten selenium is then dropped through a shot tower or by means of an eye dropper into water. The resulting pellets of selenium are then treated with petroleum ether to remove water and allowed to air dry. If desired, the pellets can also be micropulverized or worked in a mortar and pestle which reduces them to a very fine size, i. e., a particle size of about 1 to 50 microns, thus enabling the selenium to be uniformly dispersed throughout the binder material in a relatively short time. Selenium produced by this method is essentially pure amorphous selenium and if there are any other forms of selenium present, they are few in number and so fine and thoroughly dispersed throughout the amorphous selenium that they do not adversely affect the photoconducting insulating properties of the amorphous selenium or of the resulting composition.

The amount of amorphous selenium used in the composition bears a general relation to the quality of the resulting picture, since a large excess of binder material in proportion to the amount of amorphous selenium will naturally result in less selenium particles per unit area of the coating, and therefore a grainy picture, or a picture having less intensity, will result. Furthermore, if the amount of binder is much greater than the selenium, the decay or exposure rate for the coating is slower. On the other hand, there should always be sufficient binder present to effectively hold the dispersed selenium particles in the coating and to provide an adherent layer.

Compositions containing one part by volume of amorphous selenium to from 0.75 to 5 parts by volume of binder have produced good photoconducting insulating coatings on base plates. It is, however, preferred to have the estimated saturation amount of selenium in the composition, and it has been found that best results are had with a composition containing from about 1 to about 2 parts by volume of binder and about 1 part by volume of amorphous selenium. In place of amorphous selenium it is possible to substitute in the composition any other photoconducting insulating material such as sulfur, zinc titanate, anthracene, benzidine, anthraquinone, acenonaphthene, fluoranthene, naphthalene, chrysene, quinone, pyrogallic acid, microcrystalline paraffin wax, mixtures of sulfur and anthracene, and mixtures of sulfur and selenium. The photoconducting insulating material used must be such as not to cause the binder to plasticize when mixed therewith. It is preferred to use the chemically pure grade of whatever photoconducting material is employed.

The binder material should adhere tightly to the base plate on evaporation of the solvent and provide an efficient dispersing medium for the amorphous selenium particles. It should be substantially pure and the chemically pure grade of binder material is satisfactory. The binder should also have a high electrical volume resistivity so that it will not discharge the plate in the dark. To effect this result, the binder should have an electrical resistivity greater than the selenium, or other photoconducting insulating material, and greater than the base plate, and resistivity of  $10^{10}$  ohms-cm., represents about the upper practical limit possible for binders used with the base plates and photoconducting insulating materials disclosed herein. If the binder material has an electrical resistivity of less than about  $10^{10}$  ohms-cm., so little resistance is offered to the electrical charges that they tend to leak off rapidly in the dark before powder images

can be made. Excellent compositions have been obtained using materials having an electrical resistivity of from about  $10^{10}$  ohms-cm. to about  $10^{12}$  ohms-cm. The binder should not promote the formation of hexagonal selenium which is not photoconducting and insulating, nor decompose or break down during mixing or after spraying so that its electrical resistance is lowered. The binder material can be placed in the milling machinery in the size and form as commercially furnished, for it will be reduced to a very small particle size during mixing and grinding.

Satisfactory binder materials for the practice of the invention are polystyrene or Lustron manufactured by Monsanto Chemical Company, St. Louis, Missouri, Silicone (DC804) manufactured by Dow Corning Chemical Co., Midland, Michigan, Acryloid (A-10, B-72) manufactured by Rohm & Haas Company, Resinous Products Division, Philadelphia, Pa., and Vinylite (VYHH; VMCH). Vinylite (VYHH) is a vinyl-chloride-acetate resin manufactured by the Bakelite Corporation, New York, N. Y., and its approximate chemical composition is 87 per cent vinyl chloride and 13 per cent vinyl acetate. It has an intrinsic viscosity measured in cyclo-hexanone at 20° C. of 0.53. Vinylite (VMCH) is a vinyl-chloride-acetate resin which is modified with 1 per cent of an interpolymerized dibasic acid (0.7 to 0.8 carboxyl). The composition of this resin is approximately 86 per cent vinyl chloride, 13 per cent vinyl acetate, and 1 per cent dibasic acid. It has an intrinsic viscosity (cyclo-hexanone at 20° C.) of 0.53. Acryloid (A-10) is a polymerized ester derivative of acrylic and alpha methyl acrylic acids, and is supplied as a 30 per cent solids solution in Cellosolve acetate. It has a specific gravity of 1.03, a refractive index of 1.423, and a Gardner Holdt viscosity of U-W. Acryloid (B-72) is also a polymerized ester derivative of acrylic and alpha methyl acrylic acids. It is supplied as a 40 per cent solution in toluol, and has a specific gravity of 0.97, a refractive index of 1.489, and a Gardner Holdt viscosity of S-W. Silicone (DC804), a silicone resin, is supplied as a 60 per cent solids solution in aromatic naphthas and coal tar hydrocarbons (e. g. toluol, xylol, etc.). It is a straw-colored solution with a specific gravity of 1.06 and viscosity of 0.3 to 1.0 centipoise at 25° C. Polystyrene is a thermoplastic resin made by polymerizing styrene.

Parlon (chlorinated rubber) can also be successfully employed as a binder, although the addition of a small amount of a plasticizing material such as Rezyl 869 will improve its adhesion and flexibility. Parlon is chlorinated natural rubber manufactured by the Hercules Powder Company, Inc., Wilmington, Delaware. In general, this product contains from 66 to 68 per cent chlorine which corresponds approximately to the chemical formula  $(C_{10}H_{13}Cl_7)_n$ . Rezyl 869 is an alkyd resin containing approximately 60 per cent linseed oil and 40 per cent glycerol phthalate, manufactured by the American Cyanamid Company, New York, N. Y. This resin has an acid number of 2-6, contains a minimum of 27 per cent phthalic anhydride, and is supplied at 100 per cent solids. For the purposes of the invention, Parlon containing Rezyl will be considered as one binder. It is obvious that other high electrical resistance materials which form adherent layers and which do not plasticize in the presence of the selenium or adversely affect the amorphous selenium can be employed in the composition.

The solvent used should be such as to readily evaporate, and be a substantially pure, organic

low-boiling point hydrocarbon solvent, and like the binder should not introduce impurities which would lower the electrical resistance of the coating. The solvent should preferably be one that is suitable for the particular binder employed, since the solvent must not react with the binder material to form a polymerized product or similar substances which cannot be sprayed. The solvent should not affect the adhesiveness of the binder or its electrical resistance, nor should it adversely affect the pure amorphous selenium. Part of the solvent is added to the selenium and binder in the mill to provide good grinding viscosity and the balance may be added after milling to increase the fluidity of the resulting mixture. The total amount of solvent used is from about  $\frac{1}{2}$  to about 3 parts by volume of the solvent to about 1 part by volume of the binder and this proportion has resulted in readily sprayable compositions. It is preferred, however, to use from about 0.8 to about 1.4 parts per volume of solvent to about 1 part by volume of binder in the composition. Suitable solvents for use with the binders disclosed herein are toluene, Cello-solve acetate, xylene, gasline, Amsco F, benzene, methyl iso-butyl ketone or mixtures thereof.

Cellosolve acetate is an organic chemical whose formula is  $C_2H_5OCH_2CH_2OOCCH_3$ . Amsco F is an aromatic petroleum solvent manufactured by American Mineral Spirits Company, Chicago, Ill., with the following approximate characteristics: specific gravity (60° F.) 0.8628, 77 per cent aromatics, refractive index of 1.4905, mixed aniline point of 86° F., flash point 130° F., and Kouri butanol value of 70. When less solvent is present, it may be necessary to warm the composition slightly in order to spray it. The temperature of the composition should, however, not exceed 50° C. in order to obviate the production of the hexagonal form of selenium.

The base material or plate should have an electrical resistance less than either the binder material or the amorphous selenium so that it will act as a ground when the electrostatically charged coating is exposed to light. The base plate should be at room temperature and at least not above about 50° C., while being sprayed with the photoconducting insulating composition, in order to prevent formation of any crystals of hexagonal selenium in the coating which would reduce or destroy its electrophotographic usefulness. Materials having electrical resistivities of less than  $10^{10}$  ohms-cm. are satisfactory as a plate for the purposes of the invention, although it is preferred to use materials having an electrical resistivity of less than about  $10^5$  ohms-cm.

The base plate is generally flat, square or rectangular but can be of any desired shape. The surface of the plate should be cleaned before coating with the selenium composition in order to remove grease and other dirt which might prevent firm adherence of the coating to the base plate. Such cleaning can be accomplished by washing the plate with any suitable alkali cleaner, or with a hydrocarbon solvent, followed by rinsing. Any gross surface irregularities should be removed by grinding or polishing, although it is not necessary to polish the plate until it has mirror-like reflectivity. Acceptable materials for the base plate have been found to be aluminum, brass, glass, aluminum-coated glass, stainless steel, nickel, steel, bronze, copper, engraver's copper, engraver's zinc, and grained lithographic zinc, although other materials having electrical resistances similar to the aforementioned can also

be used as base plates to receive the composition coated thereon.

It is not necessary to add the selenium to the binder in the mill in the form of finely divided particles, but it can be added in the form of pellets of about  $\frac{1}{8}$ " to  $\frac{1}{4}$ " diameter. The selenium, binder and solvent should be thoroughly mixed and ground up and as a result the selenium is reduced in size and thoroughly dispersed throughout the binder or binder and solvent so that no surface irregularities or masses of unmixed particles appear in the coating on low magnification. It is preferred to mix and grind, or mill, the mass until the particles in the composition have a size less than about 50 microns, although compositions having particles up to about .0002 inch in size have proven satisfactory. Instead of adding the amorphous selenium in pellet or pulverized form to the mill, followed by separate additions of binder and solvent, a solution of the binder in the solvent can be added to the selenium in the mill. It is only essential that enough solvent be present during milling to give good grinding viscosity.

Any commercially available mixing and grinding machinery can be utilized for this step, although it is desirable to use a ball mill, and at room temperature. The mill is not heated or cooled, although while the room temperature is about 25° C., it is believed that the composition adjacent the balls may have a temperature of about 40° C. due to frictional heat developed by the balls during grinding. Ceramic, glass, or steel balls can be used in the mill. Steel balls, however, have been found best as they produce a better mixing and grinding action. The time of mixing can vary from 3 to 72 hours, although it has been found preferable to mix for about 10 to 20 hours to reduce the particles to approximately 50 microns in size. The mixing equipment should also be thoroughly cleaned before mixing to prevent the introduction of any impurities which might adversely affect the resulting selenium composition.

At the end of the milling period, additional solvent is added to the mixture and the mill operated for a short time to remove portions of the mixture adhering to the walls and balls of the mill and to enable it to be readily poured. This insures sufficient fluidity so that the composition can be easily sprayed, and provides a complete dispersion of particles in the solvent carrier or a homogenous solution or mixture. More than 90 per cent recovery of materials is thereby made possible, and while the mixture at the end of the milling period actually contains a dispersion of selenium in the binder and can be used to coat plates to provide a photoconducting insulating layer thereon, it is apparent that additional solvent is indicated as a means to facilitate spraying or coating of the plates.

Commercially available paint-spraying equipment can be used to spray the composition onto the base plate which is at room temperature. The paint-spraying mechanism should be thoroughly cleaned prior to use to prevent introduction of harmful impurities into the coating mixture. It should also provide means for heating the composition when not sufficiently fluid. The equipment should be flexible and provided with adjusting means to enable the operator to readily produce on the base plate coatings having thicknesses of from .0003 to .002 inch. Thicker coatings can be applied by longer spraying if desired, although thicker coatings increase the exposure

time for the electrophotographic plate. If the coating is too thin, pinholes are apt to occur so that a continuous film is not produced. Thus, coatings as thin as .0003 inch represent about the practical lower limit for spraying. It will be obvious to those skilled in the art that other methods besides spraying can be utilized to produce coatings of the composition on the base plate, as for example, the composition can be applied by means of a brush or draw blade, by dipping, or by roller coating.

The following examples will serve to illustrate the invention with more particularity to those skilled in the art:

*Example 1*

200 grams of pelletized amorphous, black pure selenium, 44.4 grams of Parlon, 19.2 grams of Rezyl and 90 grams of toluene were placed in a quart (Bacilli) size steel ball mill filled with  $\frac{1}{2}$  inch steel balls up to about the half-way mark and milled for about fourteen hours. After mixing, about 120 grams of additional toluene was added to the mixture to render it sprayable and the resulting red composition placed in a paint sprayer and sprayed onto a clean, flat unheated aluminum plate. As soon as the plate had been coated with a thin film of the composition about .0005 inch thick, the spraying was stopped and the coating allowed to dry by evaporation of the solvent. The hard, dry coating was completely adherent to the base plate. The plate was then charged electrostatically and used in the electrophotographic process, resulting in prints having excellent detail and no background.

*Example 2*

| Component:             | Amount, gms. |
|------------------------|--------------|
| Amorphous selenium     | 100          |
| Vinylite VYHH          | 15.2         |
| Vinylite VMCH          | 15.2         |
| Methyl isobutyl ketone | 60           |
| Toluene                | 60           |

The ingredients were charged to a pint-size glass jar approximately half filled with  $\frac{1}{2}$  inch glass balls and ground for approximately 20 hours. After milling, the mixture was drained from the jar and thinned to spray viscosity with a 50:50 mixture of toluene and methyl isobutyl ketone.

*Example 3*

| Component:        | Amount, gms. |
|-------------------|--------------|
| Vitreous selenium | 100          |
| Polystrene        | 23.8         |

The components were charged to a pint-size glass jar filled approximately half full with  $\frac{1}{2}$  inch glass balls, sufficient xylene being added to give grinding viscosity (50-100 seconds No. 4 Ford cup), and then ground for approximately 20 hours. After milling the mixture was drained from the mill and thinned with xylene to spray viscosity.

*Example 4*

| Component:        | Amount, gms. |
|-------------------|--------------|
| Vitreous selenium | 100          |
| Acryloid A-10     | 89.2         |

The components were charged to a pint-size glass jar filled approximately half full with  $\frac{1}{2}$  inch glass balls, thinned to suitable grinding viscosity with Cellosolve acetate, and ground for 72 hours. The mixture was then drained from the mill and thinned to spraying viscosity.

*Example 5*

| Component:        | Amount, gms. |
|-------------------|--------------|
| Vitreous selenium | 100          |
| Acryloid B-72     | 31.3         |
| Toluene           | 100          |

The selenium, acryloid and toluene were charged to a steel ball mill filled approximately half full with  $\frac{1}{2}$  inch steel balls and ground for 24 hours. The composition was then drained from the mill and thinned with additional toluene to spraying viscosity.

*Example 6*

| Component:         | Amount, gms. |
|--------------------|--------------|
| Amorphous selenium | 100          |
| Silicone (DC-804)  | 45.8         |

The ingredients were charged to a steel ball mill approximately half filled with  $\frac{1}{2}$  inch steel balls, toluene was then added to give suitable grinding viscosity, and the composition was ground for 42 hours. The resulting material was then drained from the mill and thinned with toluene to spraying viscosity.

X-ray studies were made of electrophotographic plates containing the photoconducting insulating coatings described herein, and revealed that some coatings appeared to contain only amorphous selenium in the binder, others apparently contained only alpha monoclinic selenium, while still others seemed to contain both amorphous and alpha monoclinic selenium dispersed throughout the binder. All of the plates, however, produced excellent powder images when used in the electrophotographic process. This appears to indicate that coatings containing the alpha monoclinic form of selenium, and those containing both the alpha monoclinic and amorphous forms of selenium are as effective as coatings containing only amorphous selenium as the photoconducting insulating material or active ingredient.

The presence of alpha monoclinic selenium in the coatings and compositions is indicated from the fact that the black, amorphous selenium mixture turned red during milling, since alpha monoclinic selenium is red although this is not conclusive because very finely divided amorphous selenium is also red. It is not thoroughly understood why alpha monoclinic selenium appears in the composition after milling, although it would appear that the milling, or the other components present during milling, or a combination of these factors, favor formation of the alpha monoclinic form. In any event, however, compositions or coatings containing only alpha monoclinic selenium as the active material, or alpha monoclinic selenium in the presence of amorphous selenium, seem to produce as effective plates as those containing essentially only amorphous selenium.

The invention teaches that electrophotographic plates can be readily produced by spraying a base plate with a composition prepared by milling amorphous selenium, a high electrical resistance binder, and a solvent, to which mixture has been added, after milling, additional solvent to render it sprayable. The finely divided particles of selenium appear to be thoroughly dispersed throughout the high electrical resistance binder and are probably coated with the binder material or substantially insulated from each other by the binder. The coated plate, or electrophotographic plate, on drying can be charged electrostatically and will hold electrostatic charges in the dark and rapidly dissipate them on exposure to light.

The invention is also applicable to the making of photocell and rectifier plates, and this application is intended to cover such modifications, departures, and adaptations as may come within the scope of the following claims.

I claim:

1. An electrophotographic plate in which the photoconducting insulating coating includes at least one material of the group consisting of

amorphous selenium and alpha monoclinic selenium in a binder comprising a continuous film of uniform thickness of thermoplastic synthetic resin which affords an effective medium which uniformly disperses said selenium and obtains good adherence of the coating to the plate, said binder having an electrical resistance higher than that of the plate and photoconducting insulating material.

2. An electrophotographic plate comprising a base plate and an adherent coating on one surface thereof, said coating comprising essentially a mixture of amorphous selenium uniformly dispersed in a binder comprising a continuous film of uniform thickness of thermoplastic synthetic resin binding together the individual particles of selenium and holding the layer on the plate, said binder having an electrical resistance higher than that of the plate and selenium.

3. An electrophotographic plate comprising a base plate and an adherent coating on one surface thereof, said coating including a mixture of alpha monoclinic selenium uniformly dispersed in a binder comprising a continuous film of uniform thickness of thermoplastic synthetic resin binding together the individual particles of selenium and holding the layer on the plate, said binder having an electrical resistance higher than that of the plate and selenium.

4. An article of manufacture consisting of a base plate and an adherent photoconducting insulating coating thereon, said coating including a mixture of equal parts by volume of substantially pure amorphous selenium uniformly dispersed in a binder comprising a continuous film of uniform thickness of thermoplastic synthetic resin binding together the individual particles of selenium and holding the layer on the plate, said binder having an electrical resistivity of from  $10^{10}$  to  $10^{19}$  ohms-cm.

5. A coated plate, the coating thereof containing essentially finely divided particles of amorphous selenium and alpha monoclinic selenium dispersed throughout a continuous phase of a binder comprising a continuous film of uniform thickness of thermoplastic synthetic resin binding together the individual particles of selenium and holding the layer onto the plate, said binder having an electrical resistivity of from  $10^{10}$  to  $10^{19}$  ohms-cm.

6. An article of manufacture comprising a base plate having an electrical resistivity less than about  $10^5$  ohms-cm. and a photoconducting insulating coating on the surface thereof, said coating including a mixture of from 1 to 2 parts by volume of a binder comprising a continuous film of uniform thickness of thermoplastic synthetic resin binding together the individual particles of selenium and holding the layer onto the plate, said binder having an electrical resistivity of from  $10^{10}$  to  $10^{19}$  ohms-cm. and 1 part by volume of at least one material of the group consisting of essentially pure amorphous selenium and alpha monoclinic selenium.

7. A composition of matter useful in the production of electrophotographic plates, including a solution of an organic, easily evaporated solvent, a binder selected from the group consisting of polystyrene, chlorinated rubber, silicone resin, acrylic resin, and vinyl-chloride-acetate resin, and at least one material of the group consisting of substantially pure amorphous selenium and alpha monoclinic selenium uniformly dispersed throughout said binder which secures together

5 the individual particles of selenium and holds the layer on the plate, the binder being substantial in volume and having a resistance higher than that of said last named material and of the plate.

8. A composition of matter including a binder comprising a thermoplastic synthetic resin having an electrical resistivity of from  $10^{10}$  to  $10^{19}$  ohms-cm., an organic, easily evaporated solvent for said binder, and finely divided particles of amorphous selenium uniformly dispersed throughout said binder.

9. A composition of matter including from 1 to 2 parts by volume of a binder comprising a thermoplastic synthetic resin having an electrical resistivity of from  $10^{10}$  to  $10^{19}$  ohms-cm., from 1.6 to 2.8 parts by volume of an easily evaporated hydrocarbon solvent for said binder, and about 1 part by volume of alpha monoclinic selenium of a particle size of from 1 to 50 microns, said selenium being uniformly dispersed throughout said binder.

10. The method of producing a composition of matter which is insulating and photoconducting and adherent after being applied as a coating to a base plate, which comprises intimately mixing and grinding in a ball mill for from 3 to 72 hours substantially pure amorphous selenium, a binder comprising a thermoplastic synthetic resin having an electrical resistivity of from  $10^{10}$  to  $10^{19}$  ohms-cm., and an organic, easily evaporated solvent.

11. In the method of producing a composition containing selenium characterized by being adherent, photoconducting and insulating after being sprayed onto a base plate and drying, the step consisting of milling in a ball mill for from 10 to 20 hours one part by volume of amorphous selenium containing not greater than about 20 parts per million of impurities and from 1 to 2 parts by volume of a binder comprising a thermoplastic synthetic resin having an electrical resistivity higher than that of the plate and selenium and selected from the group consisting of Parlon, polystyrene, silicone, acryloid, and vinylite copolymer, and an organic, easily evaporated solvent, the type of mill specified and the conditions set forth being such as not to promote crystallization of the selenium and after said milling, adding an additional amount of said solvent to the resulting mixture to provide a homogeneous mixture and to enable said mixture to be sprayed.

12. In the method of producing an electrophotographic plate, the steps comprising milling in a ball mill for from 10 to 20 hours, essentially pure amorphous selenium, an organic, easily evaporated solvent, and a binder comprising a thermoplastic synthetic resin having an electrical resistivity of from  $10^{10}$  to  $10^{19}$  ohms-cm., the type of mill specified and the conditions set forth being such as not to promote crystallization of the selenium, mixing an additional amount of said solvent in the resulting mixture to provide a homogeneous mixture and to enable said mixture to be sprayed, and then spraying the mixture containing the solvent onto a base plate, having an electrical resistivity less than about  $10^5$  ohms-cm. to provide a photoconducting insulating layer thereon.

13. In the method of producing an electrophotographic plate, the step comprising spraying a base plate at room temperature with a composition of matter including a binder comprising a thermoplastic synthetic resin having an electrical

11

resistivity of from  $10^{10}$  to  $10^{19}$  ohms-cm., a volatile hydrocarbon solvent, and at least one material of the group consisting of substantially pure amorphous selenium and alpha monoclinic selenium, said material having a particle size of from 1 to 50 microns and being dispersed throughout said binder.

ARTHUR E. MIDDLETON.

References Cited in the file of this patent 10

UNITED STATES PATENTS  
Number Name Date  
2,067,576 Mitscherling Jan. 12, 1937

12

| Name           | Date          |
|----------------|---------------|
| Gorlich        | Aug. 1, 1939  |
| Hofmann        | Oct. 31, 1939 |
| Kuymick        | Apr. 16, 1940 |
| Johnson et al. | Apr. 30, 1940 |
| Carlson        | Oct. 6, 1942  |
| Saslow         | Dec. 30, 1947 |
| Korn et al.    | Feb. 24, 1948 |
| Gray           | Oct. 25, 1949 |

## FOREIGN PATENTS

| Country | Date           |
|---------|----------------|
| Germany | Sept. 18, 1942 |